

## UNITED STATES PATENT OFFICE

2,110,281

## PURE COMPOUNDS AS EXTREME-PRESSURE LUBRICANTS

Elmer Wade Adams and George M. McNulty,  
Hammond, Ind., assignors to Standard Oil  
Company, Chicago, Ill., a corporation of Indiana

No Drawing. Application March 31, 1934;  
Serial No. 718,438

## 12 Claims. (Cl. 87—9)

This invention relates to an improved lubricant for use on bearing surfaces which are subjected to high pressures and high rubbing velocities during use.

5 The present day trend in automotive design is toward smaller rear axles and consequently smaller gears. On account of the small gears, tooth pressures and rubbing velocities are rapidly approaching a point where rear axles cannot 10 be lubricated satisfactorily with the ordinary mineral lubricating oils. The trend toward increasing loads on gear teeth in other fields has developed an urgent need for special lubricants. When hypoid gears, worm gears, heavy duty 15 bearings, planetary automatic shifts, and the like are used under conditions of high pressure and high rubbing velocities, special types of extreme-pressure lubricants must be provided in order to reduce the wear upon such moving parts. 20 Extreme-pressure lubricants are likewise important in cutting and drawing operations where the oil must withstand high pressures encountered under those conditions of use.

The object of our invention is to provide a lubricant which will give satisfactory lubrication to bearing surfaces which are subjected to high pressures and/or high rubbing velocities. A further object is to provide a lubricant which will maintain a lubricant film on bearing surfaces at 25 all times. We have found that if small amounts of certain types of organic sulfur compounds are added to the lubricating oils and soft greases, the lubricant will enable the bearing surfaces to withstand the high pressures and high rubbing 30 velocities without noticeable wear. Similarly, these sulfur compounds may be incorporated into drawing lubricants and cutting oils.

We have found that the extreme-pressure lubricants can be prepared by adding a small 40 quantity of an alkyl disulfide, high molecular weight alkyl sulfides, aryl thiocyanates and aryl isothiocyanates, xanthic disulfides, or xanthates to mineral lubricating oils, preferably, those lubricating oils having a viscosity from about 90 45 to 200 seconds Saybolt at 210° F. These compounds may be used in oils designated as S. A. E. 20, 30, 40, 50, and 60 oils. These sulfur compounds are added in quantities ranging from 1/2 to 7%, but generally amounts ranging from 1 to 50 5% are satisfactory. The organic sulfur compounds may be dissolved in the oil by any conventional mixing means. If desired, calcium and aluminum soaps or other soaps of high molecular weight fatty acids may be added to the composition to increase the viscosity or consistency 55

of the lubricant. These extreme-pressure lubricants have substantially no corrosive action upon metal surfaces.

The sulfur-bearing compounds which may be added to mineral lubricating oils or greases to 5 impart extreme-pressure lubricating properties thereto are as follows:



Wherein R and R<sub>1</sub> represent alkyl groups containing at least 5 carbon atoms each or aromatic groups such as phenyl radicals and tolyl radicals, however, when R represents a phenyl group, R<sub>1</sub> 15 may represent any alkyl group; and R<sub>2</sub> and R<sub>3</sub> represent alkyl groups or phenyl groups. The term alkyl is intended to include the saturated cyclic radicals also, such as the cyclohexyl group. Examples of the sulfides are amyl sulfide, hexyl sulfide, cyclohexyl sulfide, phenyl sulfide, ethyl phenyl sulfide, methyl phenyl sulfide, tolyl sulfide, and butyl phenyl sulfide. Examples of the 20 disulfides are ethyl disulfide, n-propyl disulfide, n-butyl disulfide, secondary butyl disulfide, tertiary butyl disulfide, cyclohexyl disulfide, ethyl propyl disulfide, amyl disulfide, heptyl disulfide, tolyl disulfide, and phenyl disulfide.



Wherein R<sub>4</sub> represents aryl groups such as phenyl, tolyl and naphthyl groups. Examples of the aryl thiocyanic esters are phenyl thiocyanic ester, tolyl thiocyanic ester, and naphthyl thiocyanic ester. Examples of the aryl isothiocyanic esters or aryl isosulphocyanic esters are phenyl isosulphocyanic ester, tolyl isosulphocyanic esters, and naphthyl isosulphocyanic ester. The aryl 35 esters of isothiocyanic acid impart excellent extreme-pressure lubricating properties to mineral oils.



Wherein R<sub>5</sub>, R<sub>6</sub>, and R<sub>7</sub> represent alkyl groups. Examples of the xanthic esters are ethyl xanthate ethyl ester, methyl xanthate ethyl ester, ethyl xanthate methyl ester, ethyl xanthate butyl ester and ethyl xanthate propyl ester. Examples of the xanthic disulfides are methyl xanthic disulfide and ethyl xanthic disulfide.

The load-carrying capacity of extreme-pressure lubricants may be determined by the extreme-pressure testing machines such as the "Almen extreme-pressure lubricant testing machine" described by Wolf and Mougey in their paper on extreme-pressure lubricants given at the 13th annual meeting of the A. P. I. at Houston, Texas, November 17, 1932.

The following table gives the load-carrying capacity of extreme-pressure lubricants as determined by an extreme-pressure lubricant testing machine designed and operated on the same principle as the Almen extreme-pressure lubricant testing machine. Those lubricants notwithstanding 15 a bearing pressure of 20,000 pounds per sq. inch are satisfactory.

Table I

Sample: 5% of the following compounds dissolved in zero bright stock (mineral oil having a viscosity of 150 Saybolt at 210° F.).

Speed of pin: 150 R. P. M.

| 25      | Compounds                   | Pressure applied per projected sq. in. in lbs. before failure | Comments |
|---------|-----------------------------|---------------------------------------------------------------|----------|
| Control |                             | About 5,000                                                   | Failed.  |
| 30      | Amyl sulfide                | 20,000                                                        | O. K.    |
|         | n-Propyl disulfide          | 25,000                                                        | Do.      |
|         | n-Butyl disulfide           | 25,000                                                        | Do.      |
|         | Diphenyl sulfide            | 20,000                                                        | Do.      |
|         | Amyl mercaptan              | 25,000                                                        | Do.      |
|         | Ethyl xanthate methyl ester | 20,000                                                        | Do.      |
|         | Phenyl isothiocyanic ester  | 25,000                                                        | Do.      |
|         | Ethyl sulfide               | 5,000                                                         | Failed   |
| 35      | Butyl sulfide               | 10,000                                                        | Do.      |
|         | n-Heptyl mercaptan          | 5,000                                                         | Do.      |
|         | Ethyl benzene sulfonate     | 10,000                                                        | Do.      |
|         | Methyl p-toluene sulfonate  | 10,000                                                        | Do.      |

As stated hereinbefore, the sulfur compounds 40 may be added to the viscous mineral oil by any suitable means. Generally the sulfur compounds are added to the mineral oil and stirred until a homogeneous mixture is obtained.

Example I

Extreme-pressure lubricants for use under conditions of high rubbing velocities and pressures can be prepared satisfactorily by mixing 5% by weight of ethyl disulfide with a mineral oil having a viscosity of about 150 to 160 Saybolt at 210° F. Coastal mineral oils, Mid-Continent oils and paraffin mineral oils may be used as the base for these extreme-pressure lubricants. Any of the hereinbefore mentioned compounds may be 55 used in the preparation of extreme-pressure lubricants instead of ethyl disulfide as set forth in Example I.

The alkyl disulfides may be prepared by any conventional means but if desired, they may be 60 prepared from the mercaptans occurring in petroleum distillates boiling within the gasoline or kerosene range. A petroleum distillate, preferably one containing a high percent of mercaptans is agitated with caustic. The caustic solution is separated from the hydrocarbon material by decantation and then oxidized with any suitable chemical reagent, for example air, or oxygen. The alkyl disulfides are then removed from the oxidized caustic solution by boiling and are collected by absorption in a mineral oil solution; if desired, they may be absorbed in the mineral oil used in the preparation of the extreme-pressure lubricant. The oxidation with air or oxygen is preferably performed under pressure and at a 75 temperature below the boiling point of the mer-

captans in the petroleum distillate. Generally this temperature is below 80 to 100° C. Other oxidizing agents such as hydrogen peroxide or potassium permanganate may be used instead of the oxygen. Also the high molecular weight alkyl disulfides may be prepared by treating hydrocarbon distillates with sodium plumbite solution and sulfur, separating the plumbite solution from the oil containing the dissolved disulfide and recovering the alkyl disulfides by distilling the hydrocarbon oil from the dissolved disulfides.

While we have described our invention with reference to particular examples, it should be understood that our invention is not limited thereby, except as set forth in the following 15 claims.

We claim:

1. An extreme-pressure lubricant comprising, a mineral lubricating oil and from  $\frac{1}{2}$  to 5% of a disulfide having the following general formula:  $R-S-S-R_1$ , wherein R and  $R_1$  represent substituents selected from the group consisting of alkyl groups or hydrocarbon phenyl groups.

2. An extreme-pressure lubricant comprising, a mineral lubricating oil and from  $\frac{1}{2}$  to 5% of 25 an alkyl disulfide having the following general formula:  $R-S-S-R_1$ , wherein R and  $R_1$  represent substituents selected from the class consisting of methyl, ethyl, propyl, butyl, amyl, hexyl, and cyclohexyl groups.

3. An extreme-pressure lubricant comprising, a mineral lubricating oil having a viscosity from 90 to 200 seconds Saybolt at 210° F. and from  $\frac{1}{2}$  to 5% of a butyl disulfide.

4. An extreme-pressure lubricant comprising, 35 a mineral lubricating oil and from  $\frac{1}{2}$  to 7% of an organic sulfide having the following general formula:  $R-S-R_1$ , wherein R and  $R_1$  represent alkyl groups containing at least 5 carbon atoms each.

5. An extreme-pressure lubricant comprising, a mineral lubricating oil having a viscosity from 90 to 200 sec. Saybolt at 210° F. and from 1 to 5% of an organic sulfide having the following general formula:  $R-S-R_1$ , wherein R and  $R_1$  represent substituents selected from the class consisting of amyl, hexyl, and cyclohexyl groups.

6. An extreme-pressure lubricant comprising, a mineral oil having a viscosity from 90 to 200 seconds Saybolt at 210° F. and from  $\frac{1}{2}$  to 5% of an organic disulfide selected from the group consisting of n-propyl disulfide, and n-butyl disulfide.

7. An improved liquid lubricant composition comprising a mineral lubricating oil and from  $\frac{1}{2}$  to 7% of a disulfide having the following general 55 formula  $R-S-S-R_1$ , wherein R and  $R_1$  represent substituents selected from the group consisting of alkyl groups and hydrocarbon phenyl groups.

8. An improved lubricant composition comprising a mineral lubricating oil and from  $\frac{1}{2}$  to 7% of an alkyl disulfide having the following general formula  $R-S-S-R_1$ , wherein R and  $R_1$  represent substituents selected from the group consisting of methyl, ethyl, propyl, butyl, amyl, hexyl and cyclohexyl groups.

9. An improved lubricant composition comprising a mineral lubricating oil and from  $\frac{1}{2}$  to 7% of an organic compound selected from the group consisting of organic sulfides having the formula  $R-S-R_1$ , wherein R and  $R_1$  represent phenyl groups or alkyl groups containing from 5 to 6 carbon atoms each; and disulfides having the general formula  $R_2-S-S-R_3$ , wherein  $R_2$  and  $R_3$  75

$R_3$  represent alkyl groups and hydrocarbon phenyl groups.

10. An extreme-pressure lubricant comprising a mineral lubricating oil and from  $\frac{1}{2}$  to 7% of an organic compound selected from the group consisting of organic sulfides having the formula  $R-S-R_1$  wherein  $R$  and  $R_1$  represent alkyl groups containing from 5 to 6 carbon atoms each and di-sulfides having the general formula  $R_2-S-S-R_3$  wherein  $R_2$  and  $R_3$  represent alkyl groups.

11. An improved lubricant composition comprising a mineral lubricating oil and from  $\frac{1}{2}$  to 7% of an organic compound, which has no cor-

rosive action upon metal surfaces, selected from the group consisting of organic sulfides having the formula  $R-S-R_1$  wherein  $R$  and  $R_1$  represent alkyl groups containing at least five carbon atoms each and di-sulfides having the general formula  $R_2-S-S-R_3$  wherein  $R_2$  and  $R_3$  represent alkyl groups.

12. An improved lubricant composition comprising a mineral lubricating oil and from  $\frac{1}{2}$  to 5% of a disulfide having the following general formula  $R-S-S-R'$ , wherein  $R$  and  $R'$  represent alkyl groups.

ELMER WADE ADAMS.  
GEORGE M. McNULTY.